# EUROPEAN PATENT SPECIFICATION

(11) **EP 0 046 826 B1**
(45) Date of publication and mention of the grant of the patent: **17.04.1985**
(21) Application number: 80302952.9
(22) Date of filing: 26.08.1980
(51) Int. Cl.: B22F 3/14, B22F 1/00, C22C 33/02

(54) **A method of drying and hot briquetting of cast iron particles**
Verfahren zum Trocknen und Heisspressen von Briketts aus Gusseisenteilchen
Procédé pour le séchage et le briquetage à chaud de particules de fonte

(43) Date of publication of application: 10.03.1982
(73) Proprietor: ECOBRIC FOUNDRY LIMITED, London, MW11 7TH (GB)
(72) Inventor: Jones, Leslie Edward, Hertford, Hertfordshire (GB); Stephens, Martin Arthur, St. Albans, Hertfordshire (GB)
(74) Representative: Freed, Arthur Woolf

## Description

This invention relates to a method of drying and hot briquetting of cast iron particles.

Within the last few years, apparatus has been devised for hot briquetting of cast iron particles such as borings. In this apparatus particles of cast iron produced for example when cast iron is machined (such borings are often known as "chips") are fed to a furnace where they are heated to the temperature at which they are plastic but not to the temperature at which they melt. Supply means are normally provided for supplying the cast iron particles to the furnace at a controlled rate and generally the apparatus also includes a vibratory screen for vibrating the cast iron particles prior to their supply to the furnace to remove undesired (tramp) particles. The hot particles are discharged from the furnace to a press where they are compacted into briquettes. The briquettes thus produced are sold to a manufacturer of cast iron and are normally remelted in a cupola or an arc or induction furnace to produce foundry castings.

In the furnace any moisture which the particles contain is vapourised and driven off as steam. Further, any oil which the chips contain also vapourises and is burnt or driven off. The percentage by weight of oil may vary enormously and the combustion of the vapourised oil does of course require some of the oxygen in the atmosphere of the furnace. The atmosphere of the furnace is desirably a reducing atmosphere in order to prevent oxidisation of the carbon in the particles as oxidisation of the carbon in the chips reduces the carbon content of the resulting briquettes below that which is desirable in subsequent use. Attempts have been made to control the air flow to the furnace to ensure that at all times the furnace atmosphere is a reducing atmosphere but difficulties have been encountered in providing adequate control and some carbon oxidation usually occurs. This problem is aggravated due to the mechanical handling of the particles by the supply means and the vibratory screen as the mechanical handling of the particles tends to remove the free carbon atoms from the particles reducing the overall carbon content of the particles. In practice, the final user of the briquettes prefers a minimum carbon level in the briquettes.

US-A-2 252 697 discloses directly reducing in finely-divided iron ore and then hot compressing and reheating the iron ore under non-oxidizing conditions followed by deformation by rolling, or forging to produce briquettes. A similar disclosure is to be found in US-A-2 457 861 which refers to the production of briquettes. There is no teaching in either of these documents of the size of the particles and although these documents refer to the addition of carbon before compression, no indication is given that it is possible to produce a high carbon material.

It is an object of this invention to provide a method of hot briquetting of cast iron particles which alleviates the problem described above.

According to this invention there is provided a method of hot briquetting of cast iron particles comprising supplying cast iron particles to a furnace in which they are heated to the plastics range and pressing the hot particles leaving the furnace into briquettes characterised, prior to the cast iron particles reaching the furnace, adding carbon particles of a diameter up to 3 mm to the cast iron particles, which have a diameter up to 9.6 mm, so that the cast iron particles are encapsulated by the carbon particles, and in that the carbon particles are added so as to constitute up to 1% by weight of the particles entering the furnace.

The addition of the carbon to the cast iron particles prior to their supply to the furnace has the advantage of increasing the carbon content in the final briquettes whatever the original carbon content and whatever the atmosphere in the furnace and has the second advantage that the additional carbon supplied tends to limit the free carbon atoms in the particles from being oxidised should the atmosphere in the furnace be an oxidising atmosphere.

Hot briquetting apparatus which utilizes a method in accordance with this invention will now be described, by way of example only, with reference to the accompanying drawing, which is a side view showing the general arrangement of the apparatus.

The hot briquetting apparatus shown in the drawing is capable of producing 5,000 kilos per hour of hot briquetted cast iron particles.

Referring to the drawing, the chips 1 are loaded into a particle loading hopper 2 by a loading crane 3 and fall into a vibratory screen 4 where tramp particles are removed; the chute through which the tramp particles fall off is denoted at 5. The particles leave the vibratory screen 4 by falling onto a conveyor 6 which convey the particles to a large storage hopper 7, capable of holding 130,000 kilos of particles. The particles fall from the hopper 7 through a manual operated feed control gate 8 onto another conveyor 9 which feeds the particles to a small supply hopper 10. The particles are fed out of the bottom of the supply hopper 10 into a screw feeder 11. The screw feeder 11 comprises a horizontal tube 12 containing an Archimedian screw driven at a variable speed. At an inlet point 13, carbon powder is metered into the tube 12 at a controlled rate. The feed tube 12 supplies the particles with carbon powder to the lower chamber 14 of a furnace 15 which functions to burn off oils in the particles and to drive off moisture. The furnace 15 contains an upper chamber 16 in which combustion of vapourised oil takes place and from which gases are exhausted into a gas stack 17.

The dried and heated particles fall from the lower chamber of the furnace through a discharge chute 18 into a briquetting press 19 of conventional construction. The briquettes fall from the press 19 onto an output conveyor 20 and are then supplied to a briquette conveyor which feeds them to a store.

The particles 1 as originally supplied are less than 3/8 of an inch mesh (9.6 mm). The carbon added is carbon 99 of up to 3 mm diameter of up to 1% by weight of the particles.

The particles entering the furnace are encapsulated in carbon powder.

Without the additional supply of carbon, the carbon content of the final briquettes would be from 2.8 to 3.2% on furnace re-melt. The additional injection of carbon changes the carbon content of the briquettes on furnace re-melt to 3.5% to 4% for example.

A typical analysis of the briquettes on furnace re-melt is as follows

The density of the finally produced briquettes is typically 80 to 84% of the engineering quality iron grade 14. The radial crush strength of a typical briquette is 1,200 to 1,500 kg/cm. The breaking load of such a typical briquette is 6,500 to 7,800 kg.

The entry point of the carbon to the apparatus is shown at 13 but could be anywhere in the apparatus.

## Claims

A method of hot briquetting of cast iron particles comprising supplying cast iron particles to a furnace in which they are heated to the plastics range and pressing the hot particles leaving the furnace into briquettes characterised, prior to the cast iron particles reaching the furnace, adding carbon particles of a diameter up to 3 mm to the cast iron particles, which have a diameter up to 9.6 mm, so that the cast iron particles are encapsulated by the carbon particles, and in that the carbon particles are added so as to constitute up to 1% by weight of the particles entering the furnace.

## Patentansprüche

Verfahren zum Heißbrikettieren von Gußeisenteilchen bei dem die Gußeisenteilchen einem Ofen zugeführt werden, in dem sie bis in den plastischen Bereich erhitzt werden, und die den Ofen verlassenden heißen Teilchen zu Briketts gepreßt werden, dadurch gekennzeichnet, daß den Gußeisenteilchen, die einen Durchmesser bis zu 9,6 mm haben, bevor die den Ofen erreichen, Kohleteilchen mit einem Durchmesser bis zu 3 mm hinzugefügt werden, so daß die Gußeisenteilchen von den Kohleteilchen umgeben werden, und daß die Zugabe der Kohleteilchen so erfolgt, daß sie bis zu 1 % (Gewichtsprozent) der in den Ofen eintretenden Teilchen ausmachen.

## Revendications

Procédé de briquetage à chaud de particules de fonte, comprenant l'amenée de particules de fonte dans un four où elles sont chauffées jusqu'au domaine plastique et la compression en briquettes des particules chaudes quittant le four, caractérisé en ce que, avant que les particules de fonte n'atteignent le four, on ajoute des particules de carbone d'un diamètre allant jusqu'à 3 mm aux particules de fonte qui ont un diamètre allant jusqu'à 9,6 mm, de sorte que les particules de fonte sont encapsulées par les particules de carbone, et en ce que les particules de carbone sont ajoutées de façon à représenter jusqu'à 1% en poids des particules pénétrant dans le four.
